

## UNITED STATES PATENT OFFICE.

WILLIAM PORTER DREAPER, OF HAMPSTEAD HEATH, ENGLAND.

## ALLOY AND ITS USES.

No Drawing. Application filed July 30, 1926, Serial No. 128,088, and in Great Britain August 5, 1925.  
Renewed February 16, 1928.

In the manufacture of jets or nozzles used for spinning artificial silk filaments or yarns or the like or where an alloy is required which is particularly hard or acid resisting or both, it is customary to use platinum or an alloy of platinum and iridium for these purposes. Where alloys of platinum and gold have been used in industry and more especially for the manufacture of the said jets, an alloy of ten per cent of platinum and ninety per cent of gold has been employed. I now find that superior results can be obtained by preparing an alloy consisting of a mixture of gold and platinum in which the latter metal is present in the proportion of from seventeen to thirty-two per cent of the weight of the alloy produced. This alloy can be prepared by melting the metals together at a temperature which allows the resulting mixture to be transferred from the crucible without any material separation of the two metals prior to or at the time of pouring and any subsequent rolling or other treating of the same.

Although I have described my invention more especially applicable to the manufacture of jets or nozzles used for spinning artificial silk filaments or yarns, I do not limit myself to this particular article as the alloy as herein set forth can be used for the manufacture of metal parts especially where acid resisting or heat resisting or special hardness or any of them is necessary.

I claim:

1. An alloy for use in the manufacture of jets for artificial silk filaments consisting of a mixture of gold and platinum, the latter metal being present in the proportion of from twenty two to twenty six per cent of the weight of the alloy produced.

2. An alloy for use in the manufacture of metal parts where acid resisting or heat resisting or special hardness or any of them is essential consisting of a mixture of gold and platinum, the latter metal being present in the proportion of from seventeen to twenty-six per cent of the weight of the alloy produced.

In testimony whereof, I have signed my name to this specification at London this 16 day of July, 1926.

WILLIAM PORTER DREAPER.